

April 18, 1939.

R. P. HEUER

2,155,165

FURNACE ROOF

Filed May 28, 1937

2 Sheets-Sheet 1



April 18, 1939.

R. P. HEUER

2,155,165

## FURNACE ROOF

2 Sheets-Sheet 2



*Witnesses:*

Elmer W. Hackel  
Walter G. Knudsen

Inventor  
Russell Pearce Heuer  
by W. Steelerson and Son  
Attorneys.

## UNITED STATES PATENT OFFICE

2,155,165

## FURNACE ROOF

Russell Pearce Heuer, Bryn Mawr, Pa.

Application May 28, 1937, Serial No. 145,357

5 Claims. (Cl. 110—99)

The invention relates to suspended basic refractory roofs for furnaces operating at high temperatures, particularly open hearth steel furnaces whose roof temperatures are in excess of 2910° F. (1600° C.).

A purpose of the invention is to improve the effectiveness of iron spacers in a suspended basic refractory roof operating at a temperature above the melting point of iron.

10 A further purpose is to use, with iron spacers in a suspended basic refractory roof, brick which have lower shrinkage than magnesia brick, but which are more resistant to spalling and more reactive with the iron spacers than ordinary chrome brick.

15 A further purpose is to employ individually hung furnace roof brick which comprise chiefly chrome ore particles imparting low shrinkage, with magnesia particles bonding the chrome ore particles and rendering them more resistant to iron oxide, and to place iron spacers laterally between the brick, which spacers oxidize and combine with the magnesia.

20 A further purpose is to prevent brick shrinkage beyond that for which thin spacers can compensate by growth through the use of a matrix of chrome larger particles, to obtain rapid oxidation and prevent melting notwithstanding that the furnace temperature is above the melting point of iron by virtue of the thinness of the spacers and to bond the chrome matrix and render it more resistant to basic oxides, and also react with the iron oxide from the spacers to form a refractory compound by use of magnesia 25 smaller particles of suitable size and in suitable proportions as later explained.

25 A further purpose is to obtain a basic suspended furnace roof of improved resistance to spalling, crushing, high temperatures and basic slags, and improved volume stability.

30 A further purpose is to employ oxidizable metal spacers having resilient prongs which removably grip the brick and hold the spacers to the brick during storage, transport and assembly.

35 Further purposes appear in the specification and in the claims.

The invention relates both to the methods involved and to the apparatus employed.

40 In the drawings one main form of the invention has been shown with desirable alternate forms, choosing the main and alternate forms primarily from the standpoints of convenience in illustration, satisfactory operation and easy demonstration of the principles involved. Brick for suspended roofs are available in such a multitude

of shapes and sizes that it is obviously impossible to illustrate all or even most of the types used.

Figure 1 is a vertical section of a typical suspended roof construction embodying the invention, the section being taken on the line 1—1 of Figure 2. Figure 1 shows the roof after assembly but before it has been subjected to furnace temperature.

Figure 2 is a sectional top plan view of the suspended roof of Figure 1.

Figure 3 is a view corresponding to Figure 1, but showing the suspended roof after it has been exposed to furnace conditions for some time.

Figures 4 and 5 are respectively front and side elevations of one of the bricks employed in the suspended roof of Figures 1 to 3 inclusive.

Figure 6 is a view corresponding to Figure 1, showing a modification of the invention.

Figures 7 and 8 are respectively front and side elevations of the spacers employed between the adjoining rear faces of the bricks of Figures 1 to 6 inclusive.

Figure 7a is a plan view of Figure 7, taken on the line 7a—7a.

Figures 9 and 10 are respectively front and side elevations of spacers used between the adjoining front faces of bricks in Figures 1 to 6 inclusive.

Figure 9a is a plan view of Figure 9, taken on the line 9a—9a.

Figures 11 and 12 are respectively front and side elevations of spacers used between adjoining side faces of the bricks in Figures 1 to 6 inclusive.

Figure 11a is a top plan view of Figure 11.

Figure 13 is a front elevation of an alternate form of brick, showing a side spacer to be used with the alternate form.

Figure 14 is a fragmentary section of Figure 13 on the line 14—14, showing a front spacer employed in connection with the brick of Figures 13 and 14.

In the drawings similar numerals refer to corresponding parts.

In referring to the unit used in constructing a suspended roof as a "brick", it is desired, of course, to include any block or similar shape, the word "brick" being employed as a convenient generic term to cover any preformed refractory shape, regardless of whether it is preliminarily fired or is subjected to furnace temperature for the first time in the furnace roof.

The present inventor has previously proposed the construction of basic suspended refractory roofs from individually hung chrome or magnesia brick laterally spaced by spacers of iron or some

5

10

15

20

25

30

35

40

45

50

55

other suitable oxidizable metal. See for example Heuer U. S. application Serial No. 707,084, filed January 18, 1934, for Suspended furnace roof. In accordance with this prior proposal of the present inventor, when the roof is subjected to furnace temperature, the metallic spacers oxidize particularly at the ends toward the furnace, and, since the oxide occupies greater volume than the original metal of the spacer, the spacers swell or grow, filling any moderate spaces left between the brick at the time the roof is constructed and compensating for shrinkage which occurs in the brick when it is heated up to furnace temperature. The compensation for shrinkage by growth of the spacer has been of primary importance where roof brick are unfired previous to being subjected to furnace temperature because the inevitable shrinkage in such unfired brick is greater than that exhibited by similar brick which have been preliminarily fired.

As a result of experiments upon the brick of the prior invention, it has been discovered that certain difficulties which may be encountered in basic suspended refractory roofs may be overcome and improvements in such roofs may be made by departing in certain respects from the prior practice. Particularly where basic suspended refractory roofs are being employed in high temperature furnaces such as open hearth steel furnaces where the roof temperature (on the side toward the interior of the furnace) is above the melting point of iron, there is considerable danger that the spacers, suitably made of iron, will melt out before they oxidize and therefore fail to perform their function of filling the space between adjoining bricks and bonding the bricks together. Especially where the unfired brick of the prior art have been used, the inevitable shrinkage of the brick is so great that the spacers must necessarily be quite thick in order to be able to compensate for the shrinkage by growth. The relatively great thickness of the spacer, while favorable from the standpoint of compensating for shrinkage of the brick, is distinctly unfavorable from the standpoint of avoiding melting of the spacer, as an unduly thick spacer, even when it oxidizes at the surface, still has a metallic core which is likely to melt.

Where the major constituent of the brick is magnesia, a relatively high shrinkage is inevitable at temperatures such as those attained by the open hearth steel furnace, and relatively thick spacers are needed to compensate for the high shrinkage. However, such relatively thick spacers do not function satisfactorily at the open hearth steel furnace temperature because they melt out between the brick.

Brick whose chief constituent is chrome ore have desirably low shrinkage at the open hearth steel furnace temperature, but in prior art practice have often been objectionable from the standpoint of low resistance to spalling and to basic oxides and failure to unite firmly in all cases with the oxidized spacer. The fact as developed by the experiments of the present inventor would seem to be that magnesia chemically combines readily with the iron oxide of the spacer, forming a compound, possibly magnesium ferrite, which is quite refractory and very strong and volume stable; whereas chrome, on the other hand, chemically unites with the iron oxide much less readily and does not appear to produce a union of as great strength as that formed with magnesia.

In accordance with the present invention, it is proposed to employ a suspended furnace roof

brick having chrome ore as its major constituent and having magnesia as its predominant minor constituent. This brick possesses a volume stability equal to or superior to that of chrome brick, thus making it possible to employ thin spacers, the spacer thickness being preferably not greater than  $\frac{3}{4}$ ths of an inch (0.109 centimeter). In resistance to spalling and to basic oxides, the brick employed in the present invention is superior to prior art chrome brick. Due apparently to its magnesia content, the brick of the present invention has the property of chemically combining readily with the oxidized spacer, in a very desirable manner to form the adjoining brick into a monolithic mass.

In this way it is possible to produce a suspended roof which is satisfactory for furnaces operating at very high temperatures, such as open hearth steel furnaces in which the temperature is in excess of  $2910^{\circ}$  F. ( $1600^{\circ}$  C.). The spacer does not melt out objectionably under open hearth steel furnace conditions apparently because, due to its thinness, it oxidizes very quickly and combines with the refractory. Due to the small brick shrinkage, the growth of the thin spacer is sufficient to fill the spaces left during construction and to compensate for the shrinkage. The brick are inherently very resistant to spalling, and spalling is further reduced by the chemical combination between the iron oxide of the spacer and the magnesia of the brick, which holds spalled fragments in place in the roof.

In order to facilitate construction of the roof, the spacers are very desirably provided with resilient prongs by which the plates can be secured to the brick before assembling the roof. One of the prongs may be the flange which has heretofore been used to prevent the spacer from dropping out of its position between the bricks. A co-operating prong desirably has contact with the hot face of the brick. After the furnace is brought up to temperature, the prongs exposed at the hot face will of course melt off, but by that time they will have performed their function.

In conventional suspended roof constructions, the bricks hang with the longest dimension generally vertical, exposing the smallest face to the furnace interior. The bricks are preferably individually hung from hangers, although of course they may if desired be hung in small groups, in which case one or more bricks of each group may be supported from other bricks. This generally used suspended roof construction may be employed in the present invention.

Where the roof is to be subjected to very high temperatures, such as those of the open hearth steel furnace, the spacers which are placed between some or preferably all of the adjoining lateral faces of the bricks will be of iron. The designation "iron" is intended to include alloys in which iron is the predominant constituent, such as steel. In furnaces operating at substantially lower temperatures than that of the open hearth steel furnace, spacers of copper or aluminum may be used, but it will be understood that iron is the preferable material for the spacers even under lower temperature conditions.

The spacers should be sheet metal of a thickness preferably not greater than  $\frac{3}{4}$ ths of an inch (0.109 centimeter), the desirable spacer thickness being  $\frac{1}{4}$ nd of an inch (0.079 centimeters). Each spacer should preferably be a single sheet in thickness, and, if the spacer in thickness comprises two or more sheets, it should

not be hollow. The cumulative effect of the oxidation and corresponding growth of the spacers is to press the bricks firmly against one another in a lateral direction, and this tightness of interfitting between the lateral faces of the bricks will increase as more and more of each spacer oxidizes, although in many instances the spacers will not oxidize all the way to the cold face of the bricks.

It will of course be understood that the present invention is not applicable to acid (silica) bricks, since these would flux the iron oxide of the spacer and destroy the roof.

Figures 1 and 2 show a typical fragment of a suspended roof structure of the present invention as it will appear after construction and before the furnace has been heated. The bricks 20 have front faces 21, rear faces 22, side faces 23, cold or top faces 24 and hot or bottom faces 25 directed toward the interior of the furnace.

The brick are individually suspended by hangers 26 engaging in recess 27 in the brick. The hangers are supported from any conventional overhead structure (suggested by hooks 26') on any suitable side structure, not shown. The hangers may if desired be supported in groups so that a particular section of the roof can be removed as a unit. If this is to be done, it may be advisable to omit spacers at the line of junction 30 between the roof units, so that lateral interlocking will not take place to prevent removal of the brick units.

In the form of Figures 1 and 2, each hanger 26 has two projections 28 and 29 which extend in opposite directions, and each of which supports an individual brick. The projections 28 and 29 engage the downwardly directed surfaces 30 of the recess 27 while the upwardly directed surfaces 31 of the recesses slope to provide clearance for, and permit ready insertion of, the projections 28 and 29. Each of the bricks is cut out at 32 to pass the body 33 of one of the hangers 26. The hangers 26 and the cooperating recesses in the bricks are conventional means for supporting a suspended roof.

If desired, the suspended roof may be surrounded by a permanent frame structure 34, of which part only is shown. Such a structure, where used, confines the brick of the roof laterally and exerts lateral pressure against adjoining brick in the roof. The frame structure 34 as shown consists of I-beams 35 and 36 joined by a strip 37 fastened at 38 to the respective I-beams. The lateral supports may be eliminated if desired, and are not present in Figure 6. A lateral thrust on the brick can be obtained by permanent expansion of the spacers without the use of lateral supports, due to the tendency of the brick to remain in vertical position under the action of gravity and due to the tendency of the hangers to remain in vertical position.

The spacers 39 are preferably of three types, which fit the peculiarities in shape of the respective faces of the brick. Each of the spacers has a flange 40, adapted to rest upon the upper face 24 of a brick as at 41 and thus prevent the spacer from dropping out of its position between the bricks before oxidation occurs to hold the spacer in place. At their ends, the flanges 40 are desirably mitered as shown at 42 to prevent the necessity of having one flange overlap another flange at a corner of the brick.

In order to prevent handling the spacers separately from the bricks at the time of assembly, 75 the spacers are desirably secured to the bricks,

as by suitable prongs. The flange 40 may be used to function as a prong at one end, while a cooperating prong 43 is placed at the opposite end of the spacer to engage the lower face 25 of the brick. The sheet iron composing the spacer is somewhat resilient so that the resilient pinching of the brick by the prongs 40 and 43 holds the spacers in place upon the brick during storage, shipment and construction of the roof. The spacer is simply snapped in place upon the brick. 10 The prongs may if desired be roughened to prevent them from slipping off the brick ends. The prong 43 is desirably mitered at 44 at the corners of the brick.

Figures 7 and 8 illustrate a spacer 45 for use 15 between the rear faces of the brick. It corresponds generally in size with the rear face 22 of the brick. Figures 9 and 10 show a spacer 46 of the same general size as the spacer 45, for use 20 between the front faces 21 of the brick. The spacer 46 is cut away at 47 to permit ready insertion of the hanger 26. Figures 11 and 12 show a spacer 48 for use between the side faces 23 of the brick.

In the form of Figures 1 to 3, the spacers will be 25 differently applied to the bricks of different longitudinal rows, the bricks of one row carrying a front face spacer and a left side spacer, while those of another row carry a rear face spacer and a right side spacer, for example. 30

It will be evident that the sizes and contours of the spacers will depend very largely upon the sizes and contours of the faces of the brick, and that, while it is desirable to have the spacers conform more or less exactly to the external outlines 35 of the brick faces, the spacers may, if desired, differ from the external outlines of the brick faces.

It will also be evident that, while Figures 1 and 2 show spacers in contact with all four lateral 40 faces of the bricks (with the exception of those bricks at the outer edges of the roof) some advantage may be obtained by using spacers between some but not all of the adjoining faces of the brick. 45

Figure 6 shows spacers between the front and rear faces 21 and 22 but not between the side faces 23 of the brick.

The hanger and spacer function may be combined in a single fitting, the detail of which is not 50 important from the standpoint of the present invention.

Figure 3 illustrates a suspended roof after it has been subjected to furnace temperature for some time. The lower ends 49 of the spacers 39 are 55 completely converted into oxide, with corresponding increase in volume, as indicated somewhat imperfectly upon the drawings. The portions of the spacers above the lower ends 49, as for example at 50, are partially converted into oxide, 60 with correspondingly less, but nevertheless marked, increase in volume. The upper portions of the spacers at 51 have not yet become very extensively oxidized. The effect of the oxidation upon the suspended roof has been to fill any 65 slight free space between the bricks left at the time the roof was constructed, to compensate for the shrinkage which occurs in the brick, to exert a lateral force between adjoining bricks and to chemically react with the adjoining brick 70 welding one brick to another by a highly refractory and very strong compound, thus producing a monolithic construction. Under the pressures developed, some of the iron oxide appears to penetrate small roughnesses in the brick surface. In 75

the great majority of the cases, all leakage openings between the brick are sealed by the growth of the spacers.

The bricks are held so firmly against lateral movement after the spacers oxidize that an individual brick may even break in pieces, and yet the pieces will not fall out. This is particularly important in the case of furnaces which are shut down from time to time, with the resultant tremendous expansions and contractions. The spacers serve to seal the roof against leakage of combustion gases or entrance of air into the furnace, thus improving the heat efficiency and prolonging the life of the furnace.

When the roof is first subjected to furnace temperature, the respective brick and spacers are relatively loose and free to move and to readjust as required by the pressure on the individual parts of the construction. Readjustment during the initial heating up of the roof is very desirable to prevent localized abnormal stresses upon individual bricks. It is only after the roof has been thoroughly heated at furnace temperature, and the action of the oxidizing atmosphere of the furnace has caused the spacers to oxidize, that the individual bricks are integrated together.

The spacers must not collapse nor compress laterally under pressure, as if they do so, they cannot by increase in volume exert lateral pressure on the bricks. Therefore each spacer should preferably comprise a single thickness of metal.

In order to indicate that various forms of brick may be used, Figures 13 and 14 show a different type of brick 20' having a recess 27' in which any suitable hanger may be inserted, and provided with spacers 52. Many variations of hangers may be used, and it is not desired to confine the present invention to constructions showing any particular type of hanger.

The brick employed in the present invention has the desirable properties of prior art chrome brick without some of the disadvantages of such prior art chrome brick. The novel brick is manufactured by employing the principle of grading the size of larger and smaller particles while omitting intermediate sized particles as previously discussed by the present inventor, and in addition, rejecting some or preferably all of the smaller chrome particles and using instead smaller magnesia particles. The use of smaller magnesia particles in preference to smaller chrome particles in a brick chiefly containing chrome ore increases the resistance to spalling, to crushing, to high temperatures and to basic slags and the volume stability beyond the properties of chrome brick of the prior art, without serious loss in density or increase in porosity.

Chrome is a satisfactory basic refractory for many purposes because of the great strength, hardness, resistance to crushing and volume stability of its particles and their chemical inertness in the metallurgical furnace. A typical analysis of chrome ore used for refractory purposes is here shown:

|                        | Per cent |
|------------------------|----------|
| Ignition loss          | 1.60     |
| Silica                 | 5.14     |
| Ferrous oxide          | 15.41    |
| Alumina                | 21.77    |
| Lime                   | Trace    |
| Magnesia by difference | 17.09    |
| Chromic oxide          | 38.99    |
| Total                  | 100.00   |

This analysis is, of course, subject to variation within the usual commercial range.

Chrome has the great advantage over magnesia that it is much less subject to shrinkage during use in the roof of a metallurgical or chemical furnace. Chrome is, however, far less basic than magnesia and much less resistant to iron oxide and other basic oxides which come in contact with the finished brick.

In the brick mix it is proposed to utilize larger particles of chrome ore in such a way as to obtain a volume stable skeleton or matrix in the brick. It is important to use chrome ore rather than magnesia as the major constituent of this matrix since magnesia exhibits an excessive shrinkage at the temperatures of an open hearth steel furnace, for example. The larger chrome particles are supplemented with additions of smaller particles of magnesia. The magnesia particles serve as a coating upon the chrome particles, bonding the chrome particles, protecting the chrome so as to make the brick more resistant to iron oxide and any other basic oxides and reacting readily with the iron oxide of the spacer. In this way the objectionable properties of chrome ore, such as its poor bonding qualities, its lack of resistance to iron oxide and other basic oxides and its lack of vigorous reactivity with the iron oxide of the spacer, are overcome and objectionable features of magnesia, such as its tendency to shrink excessively at the temperature of the open hearth steel furnace, are also not harmful.

For the smaller particles magnesia which is desirably the calcined or dead-burned magnesite or periclase of usual commercial grade is employed. Typical analyses follow:

|                        | Percent | Percent | 40 |
|------------------------|---------|---------|----|
| Ignition loss          | 0.00    | 0.10    |    |
| Silica                 | 0.67    | 3.36    |    |
| Ferric oxide           | 7.13    | 1.46    |    |
| Alumina                | 0.25    | 1.02    |    |
| Lime                   | 2.29    | 1.11    |    |
| Magnesia by difference | 89.66   | 92.95   |    |
| Total                  | 100.00  | 100.00  | 45 |

These analyses are, of course, subject to variation within the usual commercial range, and higher lime content, in some cases as much as approximately 20%, may be present in the magnesia if the use of such impure magnesia is desired.

From the standpoint of resistance to spalling, resistance to crushing, volume stability and resistance to high temperature, the use of chrome particles of optimum size is important. The chrome particles should range in size between 3 and 20 mesh per linear inch, and may very desirably be more closely graded as to size, for example ranging between 6 and 20 mesh per linear inch, between 3 and 10 mesh per linear inch, or between 3 and 6 mesh per linear inch, etc.

Of course it will be understood that no commercial screening process is one hundred percent efficient and that, notwithstanding due care, chrome particles commercially produced to range in size between 3 and 20 mesh per linear inch, 6 and 20 mesh per linear inch, 3 and 10 mesh per linear inch, 3 and 6 mesh per linear inch, etc., will have a certain small proportion, possibly as much as 10% or even in an extreme case 15% in the dry mix, of chrome particles of smaller size. Likewise, there may be a small proportion, possibly 1% or 2% or even in an extreme case 5% in the dry mix, of chrome particles of larger size.

Based on the weight of the refractory, there may be as much as 15% of the larger particles outside the chosen size range due to the inefficiency of commercial screening. This will be made clear by the following typical screen analyses of chrome particles commercially graded to be between 6 and 20 mesh per linear inch in one case, between 3 and 10 mesh per linear inch in another case, and between 3 and 6 mesh per linear inch in another case:

| Mesh per linear inch | 6 x 20  | 3 x 10  | 3 x 6   |
|----------------------|---------|---------|---------|
|                      | Percent | Percent | Percent |
| 15 On 3              | Nil     | 1       | 2       |
| Through 3 on 4       | Nil     | 13      | 36      |
| Through 4 on 6       | 1       | 27      | .56     |
| Through 6 on 8       | 23      | 29      | 4       |
| Through 8 on 10      | 26      | 18      | 2       |
| Through 10 on 14     | 26      | 7       | Nil     |
| Through 14 on 20     | 21      | 5       | Nil     |
| Through 20           | 3       | Nil     | Nil     |
| Total                | 100     | 100     | 100     |

The intermediate size particles are omitted or the quantity of intermediate sized particles is maintained very low.

The magnesia smaller particles should pass 48 mesh per linear inch. They have the following typical screen analysis:

| Mesh per linear inch | Per cent |
|----------------------|----------|
| On 35                | Trace    |
| Through 35 on 48     | 2        |
| Through 48 on 65     | 10       |
| Through 65 on 100    | 16       |
| Through 100          | 72       |
|                      | 100      |

It will of course be evident that the fineness of the smaller particles may be increased, using smaller particles for example passing entirely through 65 mesh per linear inch, or even smaller.

Of the chrome larger particles, between 65% and 75% (that is, between 65 and 75 parts in 100 parts) are employed, preferably using about 70%. Of the magnesia smaller particles, between 35% and 25% (between 35 and 25 parts in 100 parts) are employed, preferably using about 30%.

To a slight extent chrome may be substituted for magnesia and magnesia for chrome without affecting the special properties of the brick, although the larger particles will be chiefly or predominantly chrome and the smaller particles chiefly or predominantly magnesia. This means that more than 50%, most desirably 100%, of the larger particles will be chrome ore, and more than 50%, most desirably 100% of the smaller particles will be magnesia. The larger particles will preferably comprise in excess of 80% chrome and not over 20% magnesia, while the smaller particles will preferably comprise in excess of 80% magnesia and not over 20% chrome. This will be understood when reference is made in the claims to larger particles of chrome and smaller particles of magnesia.

Conventional brick-making practice is used as far as the preparation of the brick mix is concerned. The larger chrome particles and smaller magnesia particles are mixed with water, preferably adding enough water to temper the mix, desirably about 2% based on the weight of the wet mix.

Where the brick is to be kiln fired as later explained, it is not necessary to use a bonding substance. If it is preferred, however, to make a

brick which is suitable for use without previous kiln firing, a bonding substance should be employed.

As a bonding substance, sulphuric acid may be used. One suitable mix might be bonded with about 1% of 66° Baumé sulphuric acid based upon the weight of the wet mix (the percentage is practically the same if based on the dry finished brick). As much as 2% or even more of sulphuric acid may be used. Where sulphuric acid of another strength is used, allowance should be made in the percentage employed. For some uses clay may be added as a bond, and as much as 2% or less desirably even 5% of clay may be added if desired in addition to the sulphuric acid.

Other bonding substances such as sodium acid sulphate, sodium silicate or organic bonding substances like waste liquors from the sulphite paper process, dextrin, etc., may be used. The quantity of sodium acid sulphate, sodium silicate or organic bonding substance will most desirably be limited to 1% or permissibly 2% of the wet mix, not considering in this 2% the water which is used to dissolve the bonding substance. In any case the quantity of any such bonding substance will not exceed 5% of the wet mix. Clay, preferably not exceeding 2% but less desirably up to 5% of the wet mix, may be used with any of the above bonding substances.

The total bonding substance will very desirably be limited to 5% of the wet mix so as not to impair the refractory properties of the brick. The bonding substance may be mixed with the tempering water before incorporating the water in the mix.

The moistened brick mix is molded under a pressure exceeding 1000 pounds per square inch (70.3 kilograms per square centimeter), preferably exceeding 5000 pounds per square inch (351.5 kilograms per square centimeter), and most desirably exceeding 10,000 pounds per square inch (703 kilograms per square centimeter). It is preferable to apply a vacuum during the molding, increasing the pressure in a second step after the vacuum is applied.

The molded brick, if they are to be kiln fired, are dried preparatory to kiln firing, and then fired, suitably at a temperature such as 1830° F. (1000° C.) or above, for example 2190° F. (1200° C.) or 2730° F. (1500° C.). Where a bonding substance has been used, the brick need not be kiln fired, but should be treated to develop the bond, after which they may be shipped in unburned condition and subjected to firing temperature for the first time in the metallurgical or chemical furnace in which they are used. The preferred treatment to develop the bond is to heat the moist brick to a temperature between 212° and 572° F. (100° and 300° C.) until substantially all free moisture is removed. The dry brick are then ready for use.

The excellent properties of the brick of the present invention are indicated by the following data for the unfired brick, it being understood that the obtaining of such properties is more of an achievement in an unfired brick than in a fired brick, but that the properties obtainable for the fired brick are generally as good as those for the unfired brick.

Although density is not the prime consideration in the present invention, the brick of the present invention when bonded and in unfired condition, after drying for 75 hours at 25° F. (12.5° C.), has a bulk specific gravity in excess of 3.10, prefer-

ably about 3.20. The open pore space is less than 10%.

A very high resistance to spalling is obtained in the actual finished brick as indicated by tests 5 under conditions of actual use. The cold crushing strength of the dry unfired brick exceeds 2000 pounds per square inch (140.5 kilograms per square centimeter) and often exceeds 4,000 pounds per square inch (281 kilograms per square 10 centimeter).

The brick of the present invention in unfired condition is very volume stable and has excellent resistance to high temperature, as indicated by the fact that when reheated in a testing furnace 15 to 3200° F. (1815° C.) for 24 hours or more the brick show a change in linear dimensions of less than 1% shrinkage.

Tests under actual conditions of use indicate 20 very high resistance to basic slags and other basic oxides.

The efficiency of the sulphuric acid bond depends of course upon the presence of magnesia smaller particles and is slightly diminished by substitution of chrome smaller particles for magnesia. The bond, after it is once developed, is 25 effective at ordinary room temperatures and is supplemented after the brick are heated to firing temperature during use, by a reaction between the constituents of the brick. The excellent service 30 characteristics of the brick of the present invention, and particularly the resistance to spalling, crushing, high temperatures and basic slags, and the volume stability, are due in part to the tight interfitting between particles, to the presence of an optimum size of chrome particles, to the presence of the magnesia smaller particles and to the presence of an optimum proportion 35 and optimum size of magnesia particles.

The magnesia in the brick is important not 40 only from the standpoint of the properties of the brick itself, but also in order to render the brick capable of reacting readily with the oxide of the spacer metal to unite the brick firmly to the spacer by a compound which is refractory 45 and volume stable under the furnace conditions and which makes of the roof effectively a monolithic structure.

Where reference is made to a sulphate acid bonding substance it is intended to include both 50 sulphuric acid and acid sulphates such as sodium acid sulphate.

The screens which have been described as possessing certain mesh per linear inch are Tyler Standard screens.

Commercial screening frequently employs screens which are inclined at an angle from the horizontal and have rectangular openings. These screens should be chosen so that the particles which are produced, when tested by screening 60 over standard screens, shall conform to the required grading.

All percentages mentioned herein are percentages by weight unless otherwise indicated by the context. Open pore space or porosity is of course 65 expressed as percentage by volume. The percentages of the chrome and magnesia particles are percentages by weight based upon the dry mix. They may also be expressed as parts instead of percentage. The percentages of water and bonding substance are percentages by weight based 70 upon the wet mix. The screen analyses are expressed in percentages by weight based upon the total material being analyzed.

Percentages based upon the dry mix are sub- 75 stantially identical for practical purposes with

percentages based upon the dry finished brick, and one can be used as the other without change if desired.

In view of my invention and disclosure variations and modifications to meet individual whim or particular need will doubtless become evident to others skilled in the art, to obtain all or part of the benefits of my invention without copying the structure shown, and I, therefore, claim all such in so far as they fall within the reasonable 10 spirit and scope of my invention.

Having thus described my invention, what I claim as new and desire to secure by Letters Patent is:

1. In a refractory roof, a plurality of suspended 15 refractory bricks positioned side by side, supported by hanging from above, having lateral faces which are adjacent and generally parallel and comprising chiefly chrome ore with magnesia as the chief minor constituent, and spacers 20 between lateral faces of the bricks, each spacer contacting the refractory material of the generally parallel faces of adjacent bricks, the spacers comprising iron part at least of which is oxidized and iron oxide of the spacers being combined 25 with the magnesia of the bricks on both sides of individual spacers.

2. In a refractory roof, a plurality of suspended 30 refractory bricks positioned side by side, supported by hanging from above, having lateral faces which are adjacent and generally parallel and comprising chiefly chrome ore in the form of relatively larger particles with magnesia in the form of relatively smaller particles interspersed among and coated on the larger chrome 35 particles, and spacers between the lateral faces of the bricks, each spacer contacting the refractory material of the generally parallel faces of adjacent bricks, the spacers comprising iron part at least of which is oxidized and iron oxide of the 40 spacers being combined with the magnesia of the bricks on both sides of individual spacers.

3. An open hearth steel furnace roof having a plurality of volume-stable chrome-magnesia suspended 45 refractory bricks positioned side by side, supported by hanging from above, having lateral faces which are adjacent and generally parallel and containing more than 50% chrome ore, and sheet iron spacers between the lateral faces of the bricks, each spacer contacting the refractory 50 material of the generally parallel faces of adjacent bricks, said spacers being not greater than  $\frac{3}{64}$ ths inch in thickness and being adapted to oxidize and combine with the magnesia of the bricks on the two sides of each spacer rather than 55 melt out when the open hearth is brought up to operating temperature.

4. In a suspended furnace roof, a plurality of suspended refractory bricks positioned side by side, having lateral faces which are adjacent and 60 generally parallel and comprising more than 50% chrome ore with magnesia as the chief minor constituent, means for individually hanging the bricks from above and spacers between lateral faces of the bricks, each spacer contacting the 65 refractory material of the generally parallel faces of adjacent bricks, the spacers comprising iron part at least of which is oxidized and iron oxide of the spacers being combined with the magnesia of the bricks on both sides of individual spacers. 70

5. In a suspended refractory roof, a plurality of dry chrome-magnesia suspended refractory bricks positioned side by side, supported by hanging from above, having lateral faces which are adjacent and generally parallel and comprising 75

tightly interfitted masses of from 65 to 75 parts of larger particles consisting chiefly of chrome ore and large enough to be retained on a 20 mesh per linear inch screen and from 35 to 25 parts of smaller particles consisting chiefly of magnesia and small enough to pass through a 48 mesh per linear inch screen in combination with spacers between the lateral faces of the bricks,

each spacer contacting the refractory material of the generally parallel faces of adjacent bricks, the spacers comprising iron part at least of which is oxidized and the iron oxide of the spacers being combined with the magnesia of the bricks on both sides of individual spacers.

RUSSELL PEARCE HEUER.